

## UNITED STATES PATENT OFFICE

2,306,017

## POUR POINT DEPRESSANT FOR LUBRICATING OILS

Jacob Faust, Belleville, N. J., assignor to L. Sonnenborn Sons, Inc., a corporation of Delaware

No Drawing. Application December 31, 1940,  
Serial No. 372,485

1 Claim. (Cl. 252—35)

This invention relates to new and useful improvements in pour point depressants for lubricating oils.

Pour point depressants have in the past been used in connection with waxy petroleum hydrocarbon oils having a relatively high pour point due to the wax contained therein. The use of these depressants, however, is attended by the disadvantage that the pour point obtained, though in many cases materially depressed, is substantially fugitive and reverts upon storage or in service progressively towards the pour point of the original undepressed oil.

I have discovered that this disadvantage may be overcome and that a substantially permanent lowering of the pour point and a substantially non-fugitive, non-reverting pour point may be obtained by admixing with the oil tin stearate.

For the purpose of depressing the pour point of a paraffin base oil, such as a Pennsylvania grade oil, in accordance with the invention, so much tin stearate is added thereto as is sufficient to appreciably reduce the pour point of the oil and preferably reduce the same at least 10° below its normal pour point. 0.01 to 1.0% will give satisfactory results in most cases. 0.2% tin stearate constitutes usually the maximum amount for the procurement of maximum depression. Above 0.25% the depression obtained by the stearate will progressively decrease until it approaches the value of 0.01% addition at about 1.0%. The preferred amount within the specified range is 0.2% tin stearate, which will yield maximum depression.

Though satisfactory depression is obtained within the broad ranges of 0.01 to 1.0% of tin stearate, not all additions within that range will give satisfactory stable non-reverting pour points. I have discovered that when using less than substantially 0.1 and in excess of substantially 0.75% tin stearate, the primary pour points obtaining in the oil will exhibit a tendency to revert and is of a substantially fugitive character. When, however, limiting tin stearate additions to the 0.1 to 0.75% range, substantially stable non-fugitive and non-reverting points are procured.

In the following table various tin stearate concentrations in a Pennsylvania grade S. A. E. 20 oil are illustrated reciting in the respective columns concentration of stearate, primary pour point, the absolute reduction obtained, and the secondary pour point measured in accordance with reversion tests:

Table I

| SAE 20<br>(orig. P. P. +30) | Primary<br>P. P. | Absolute<br>reduction |     | Second-<br>ary P. P. |
|-----------------------------|------------------|-----------------------|-----|----------------------|
|                             |                  | °F.                   | °F. |                      |
| SAE 20 plus—                |                  |                       |     |                      |
| 0.01%                       | +20              | 10                    | +20 |                      |
| 0.05%                       | -5               | 35                    | +10 |                      |
| 0.1%                        | -10              | 40                    | -10 |                      |
| 0.15%                       | -15              | 45                    | -15 |                      |
| 0.2%                        | -20              | 50                    | -20 |                      |
| 0.25%                       | -15              | 45                    | -15 |                      |
| 0.5%                        | -10              | 40                    | -10 |                      |
| 0.75%                       | +10              | 20                    | +15 |                      |
| 1.0%                        | +25              | 5                     | +25 |                      |
| 2.0%                        | +35              |                       | +40 |                      |
| 5.0%                        |                  |                       |     |                      |

In all cases the oil depressed with tin stearate showed appreciable depression, i. e., at least 10° from the original pour point of the oil plus 30° F. In concentrations below 0.1% and above 0.75% the pour point was substantially stable, whereas above and below these concentrations the same was fugitive. The pour point measurements were carried out as by the A. S. T. M. tests for the determination of pour point designated as D97-39. The reversion data cited in the table were obtained by storing the oil at 32° F. for 168 hours and observing the temperature at which the oil loses fluidity.

In the following Table II a series of pour point reversion tests are tabulated for a variety of Pennsylvania grade oils:

Table II

| Penn.<br>grade oil<br>(original<br>pour<br>point—<br>25° F.) | Concentration<br>tin stearate | Primary<br>pour point | Secondary<br>pour point | Rever-<br>sion |
|--------------------------------------------------------------|-------------------------------|-----------------------|-------------------------|----------------|
| SAE 10...                                                    | 0.2% tin stearate             | —20                   | —20/-15                 | 0              |
| SAE 20...                                                    | do                            | -15                   | -15/-10                 | 0              |
| SAE 20...                                                    | do                            | -5                    | -5/-10                  | 0              |
| SAE 20...                                                    | 0.25% tin stearate            | -10                   | -5/-10                  | 0              |
| SAE 40...                                                    | 0.2% tin stearate             | 0/-5                  | 0/-5                    | 0              |
| SAE 40...                                                    | 0.25% tin stearate            | -5/-10                | -5                      | 0              |

For best results it is essential that the tin stearate to be incorporated in a given Pennsylvania grade oil in accordance with the invention is one which will yield substantially clear solutions in the oil. If a product is used which does not satisfactorily form substantially clear solutions in the oil to be depressed, its efficiency, both as to reduction of pour point and as pour point reversion tendency will be found impaired, if not altogether 0. This is particularly true of products during the manufacture of which

oxidative or other detrimental influences have been permitted to disturb or negative the reaction designed to lead to the intended tin stearate product.

I find it of advantage and use a tin stearate product substantially obtained by fusing a freshly precipitated stannous hydroxide (precipitated, for instance, with ammonia from aqueous stannous salt solutions preferably in an inert atmosphere such as  $\text{CO}_2$ ) with stearic acid at approximately  $340^{\circ}\text{ F}$ . in substantially stoichiometrical proportions (calculated on  $\text{Sn}(\text{stearate})_2$ ). The reaction should preferably be carried out in an inert atmosphere such as an atmosphere of  $\text{CO}_2$  or the like.

The foregoing description is by way of illustration and not of limitation and I am not to be

limited to any details but only by the appended claim in which I have endeavored to claim broadly all inherent novelty.

I claim:

A lubricating oil composition of relatively low, substantially non-fugitive, non-reverting pour point comprising a wax-containing petroleum hydrocarbon oil having normally a relatively high pour point due to the wax contained therein, and 0.1 to 0.75% of a stannous stearate obtained by fusing together freshly precipitated stannous hydroxide with stearic acid in an inert atmosphere, said stannous stearate being substantially soluble in said hydrocarbon oil to form substantially clear solutions therein.

JACOB FAUST.